

## UNITED STATES PATENT OFFICE

2,604,391

GAS-PRODUCING NONDETONATING  
COMPOSITION

James Taylor and Alexander Cantlay Hutchinson, Saltcoats, Scotland, assignors to Imperial Chemical Industries Limited, a corporation of Great Britain

No Drawing. Application June 24, 1949, Serial No. 101,273. In Great Britain November 8, 1946

5 Claims. (Cl. 52-7)

1

The present invention relates to new or improved gas-producing charges of the kind capable of propagating a self-sustained gas-producing non-detonating decomposition throughout themselves, when they are locally heated by a limited non-detonating igniting element; that is to say, one capable of heating a small portion of the charge to a high temperature and insufficient of itself to effect any substantial general rise in the temperature of the charge.

Depending on the rate at which the gas-producing decomposition is propagated throughout the charge under increasing pressure conditions, the nature of the gases produced, the amount and quality of any solid products of the reaction and the presence or absence of flame, such charges find application for a variety of purposes, including, for instance, the generation of gas pressure for actuating pneumatically operated mechanical devices and blasting operations when a slow heaving action is required, as in the winning of lump coal.

This application is a continuation-in-part of applicants' copending application Serial No. 774,693, filed September 17, 1947, now abandoned.

It is known in the art that guanidine nitrate and nitroguanidine may be decomposed when strongly heated, giving a good yield of permanent gases that would be suitable for the aforesaid purposes leaving a certain amount of solid residue.

U. S. Patent No. 2,159,234, discloses a composition which may be used as a non-detonating, gas generating composition capable of undergoing a self-sustaining decomposition without detonation. This composition comprises at least one substance selected from the group consisting of ammonium nitrate, guanidine nitrate, urea nitrate and dicyandiamidine nitrate; a carbonaceous material; and from 1 to 20% of a sensitizing agent comprising at least one member of the group consisting of chromic oxide, alkali metal chromates, ammonium chromate, ammonium dichromate and alkali metal polychromates. If a cooling salt is included in the composition, the composition may be employed for blasting purposes in a pressure operated device having in combination a pressure resistant, pressure responsive container, and deflagrating ignition means. When guanidine nitrate is sensitized by the presence of a suitable proportion of a chromate or bichromate, the decomposition of a charge of the mixture which has not previously been heated, will sustain itself throughout the entire charge once it has been excited by temporary heating of a

2

local portion of the charge as by means of a limited heating element such as an electric powder fuse or a red hot rod even at ordinary pressure.

5 The composition taught in U. S. Patent No. 2,159,234 which could consist of guanidine nitrate, a carbonaceous material, and from 1 to 20% of a chromate or dichromate has the disadvantage that it requires a relatively large amount 10 of the chromate or dichromate in order to produce a composition which will burn at a high rate and still produce a gas under low pressure. The inclusion of a high percentage of a chromate or dichromate dilutes the gas-producing compound, guanidine nitrate, to such an extent 15 that a large amount of residue remains after ignition of the composition. If, for example, such a composition were utilized for thermally vaporizing a pesticidal compound, unburned ash resulting from the presence of the chromate or dichromate would exist and could be clearly objectionable. Furthermore, the use of a chromate or dichromate sensitizer with guanidine nitrate does not produce a composition having a 20 sufficiently high burning rate to vaporize, for example, a pesticidal compound in a short time as might be required in fumigating open areas in the field. If the pesticide in this case were not vaporized quickly, it should be evident that the pesticidal compound would be dispersed by the wind or other elements prior to the time that a sufficient 25 concentration of the vaporized pesticide could be built up to accomplish its purpose. Other uses for which higher burning rates at increased pressures might be required have necessitated further research by the applicants. It is the result 30 of this research that has brought the present invention into being.

An object of the present invention, therefore, is the provision of improved charges for gas pressure operated devices which charges include compositions capable of undergoing a self-sustained, gas-producing, non-detonating decomposition when ignited with the aid of a local and limited heating element.

A further object of the present invention is to produce a charge of the aforesaid characteristics which has a relatively high burning rate compared with those compositions previously produced by the teaching of the prior art.

Another object of this invention is to produce a composition which is not only of a higher relative burning rate but which also, upon decomposition, evolves a higher yield of permanent gases than would be possible upon the decomposition

of the prior arts compositions and which evolve this higher yield of gases without leaving a large amount of residue as do the compositions of the prior art.

Further objects of this invention will become apparent upon consideration of the description of the invention hereinafter.

Applicants have found that copper powder and copper compounds in pulverulent condition act as sensitizers for the thermal decomposition of nitroguanidine and guanidine nitrate, thereby enabling the production of new or improved charges suitable for the aforesaid purpose and capable of decomposing with the evolution of a high yield of permanent gases at a higher rate of evolution even at low pressures without leaving a residue of objectionable unburnt components of the sensitizers.

According to the present invention, therefore, a gas-producing charge of the kind suitable for carrying out the objects of this invention comprises a composition of which the preponderating constituent is at least one nitrogen containing compound selected from the group consisting of nitroguanidine and guanidine nitrate and in admixture with said compound a copper containing pulverulent sensitizer for the thermal decomposition of said compound selected from the group consisting of copper powder, cupric oxide, cuprous chloride and cuprous oxydate. Other copper compounds may be utilized but preferably those which are non-hygroscopic are the ones preferred in this invention. In certain instances, when cuprous chloride is used as a sensitizing agent, a slight amount of chlorine is evolved. In engine driving, for example, this is objectionable and copper oxide is preferably employed instead of cuprous chloride as a sensitizing agent.

Certain compounds of vanadium may desirably be utilized along with cuprous chloride for the purpose of further increasing the rate of burning of the composition. Vanadium pentoxide in an amount of 1% when added to mixtures of guanidine nitrate or nitroguanidine sensitized by cuprous chloride causes a marked increase in the rate of burning.

Charges made in accordance with this invention decompose smoothly when they are ignited, and in compressed condition, they do not undergo discontinuous volume changes at temperatures at which they are likely to be exposed on storage. It is further possible, according to the invention, to obtain charges that decompose without flame when they are locally heated and which are, accordingly, suitable for blasting in fiery or dusty mines. For blasting purposes, it is frequently desirable to confine the mixture in order to enable the pressure to be built up satisfactorily and for this purpose, a blasting assembly comprising a gas-producing charge confined in a pressure resisting vessel having the closure adapted to yield at a predetermined pressure may conveniently be employed.

The invention is illustrated in the following examples in which the parts are parts by weight of the total composition.

#### Example 1

98 parts of guanidine nitrate and 2 parts of cuprous chloride are mixed together in a mechanical mortar. The resulting mixture is pressed and this product is broken down into grains of a size 4/24 B. S. S. units. 200 grams of these grains when decomposed in a steel tube blasting device 3 feet long by 1 1/4 inches internal diameter

burst a disc 7/16 inch thickness. An electric powder fuse containing 60 grains of black powder is used to excite the decomposition.

#### Example 2

A mixture consisting of 97 parts of guanidine nitrate and 3 parts of cuprous chloride was prepared by milling the powder in a ball mill until an intimate mixture was obtained. A quantity of this mixture was pressed in the form of a pellet in a hydraulic press. The sensitized charge so formed was found to be capable of decomposition in a self-sustained manner when ignited by the application of heat and it had a burning rate of 0.038 inch per second at a pressure of 125 pounds per square inch.

The addition of a small percentage of vanadium pentoxide (1%) when added to the above mixture of guanidine nitrate sensitized by cuprous chloride caused a marked increase in the rate of burning.

#### Example 3

For the purpose of comparing the compositions of U. S. Patent 2,159,234 with the present invention, a mixture of guanidine nitrate sensitized by ammonium dichromate was prepared. This mixture consisted of 90 parts of guanidine nitrate and 10 parts of ammonium dichromate made up in the form of Example 2. When ignited by the application of heat, it had a burning rate of only 0.028 inch per second at a pressure of approximately 100 pounds per square inch.

#### Example 4

20 parts of cuprous chloride and 80 parts of guanidine nitrate are mixed together in a mechanical mortar. 200 grams of this mixture when decomposed in a steel tube blasting device 3 feet long by 1 1/4 inches internal diameter bursts a disc 7/16 inch thickness. An electric powder fuse containing thirty grains black powder is used to excite the decomposition.

It is noted that in this example, a much higher percentage of cuprous chloride is present as a sensitizer for guanidine nitrate than in Example 1. The bursting power for a disc in the two examples is the same. However, in Example 1, the preferred ratio of cuprous chloride to guanidine nitrate is employed and as a result, relatively no residue is present after decomposition of the mixture in Example 1 as compared with the residue present upon decomposition of the composition of this example.

Whereas it has been indicated that both nitroguanidine and guanidine nitrate may be sensitized by a small amount of a copper-containing compound, there are advantages in particular instances in using nitroguanidine in preference to guanidine nitrate and in other instances in using guanidine nitrate in preference to nitroguanidine. Guanidine nitrate is cheaper than nitroguanidine, it is non-explosive, and has better pressing properties. However, nitroguanidine compositions are relatively non-hygroscopic in comparison with guanidine nitrate compositions. Also, nitroguanidine sensitized compositions generally produce hotter gases than the guanidine nitrate compositions. If, therefore, it is desirable to have a composition relatively less hygroscopic or if it is desired to have a composition which produces hotter gases, nitroguanidine is the preferred compound to be sensitized. In all other cases, considering cost, non-explosive qualities and better pressing properties, it is more desirable to use guanidine nitrate.

We claim:

1. A gas-producing charge of the type herein defined consisting essentially of at least one nitrogen-containing compound selected from the group consisting of nitroguanidine and guanidine nitrate and 2 to 20% by weight of a pulverulent copper-containing sensitizer selected from the group consisting of copper, cupric oxide, cuprous chloride, and cuprous oxylate.

10 2. A gas-producing charge as set forth in claim 1 wherein the sensitizer comprises cuprous chloride.

15 3. A gas-producing charge of the type herein defined consisting essentially of at least one nitrogen-containing compound selected from the group consisting of nitroguanidine and guanidine nitrate; 2 to 20% by weight of a pulverulent copper-containing sensitizer selected from the group consisting of copper, cupric oxide, cuprous chloride, and cuprous oxylate; and a small percentage of vanadium pentoxide.

20 4. A gas-producing charge as set forth in claim 3 wherein the sensitizer comprises cuprous chlo-

ride and the vanadium pentoxide is present in proportion of 1% by weight.

5 5. A gas-producing charge of the type herein defined consisting essentially of guanidine nitrate and 2 to 20% by weight of a pulverulent copper-containing sensitizer selected from the group consisting of copper, cupric oxide, cuprous chloride, and cuprous oxylate.

JAMES TAYLOR.

ALEXANDER CANTLAY HUTCHISON.

#### REFERENCES CITED

The following references are of record in the file of this patent:

#### UNITED STATES PATENTS

| Number    | Name   | Date         |
|-----------|--------|--------------|
| 2,159,234 | Taylor | May 23, 1939 |

#### FOREIGN PATENTS

| Number | Country       | Date |
|--------|---------------|------|
| 21,189 | Great Britain | 1902 |